

## UNITED STATES PATENT OFFICE

2,365,974

## TREATMENT OF HYDROCARBON OIL

William Schreiber, Philadelphia, Pa., assignor to  
 The Atlantic Refining Company, Philadelphia,  
 Pa., a corporation of Pennsylvania

No Drawing. Application May 21, 1943,  
 Serial No. 487,971

18 Claims. (Cl. 252—53)

This invention relates to a method for producing improved lubricating oils, and more particularly to a method for producing lubricating oils having increased film-strength and increased resistance to oxidation and sludging. The invention constitutes an improvement over the method of treating lubricating oils described in United States Patent 2,220,851, issued to me on November 5, 1940.

In the identified United States patent, I describe a process for preparing improved lubricating oils which comprises subjecting a mixture of a hydrocarbon lubricating oil, which is usually an oil having a high viscosity index, and an organic compound of trivalent phosphorus to a thermal treatment in the presence of an artificially or extraneously introduced oxidizing agent, such as air or other oxygen-containing gas, for a period of time sufficient to cause the formation of phosphorus-containing reaction products, some of which are soluble and some of which are insoluble in the oil. The process further comprises the separation of the insoluble portion of the phosphorus-containing reaction products before application of the oil as a lubricant either per se or in the form of a blend with untreated oil.

The many organic compounds of trivalent phosphorus which may be reacted with a hydrocarbon oil in accordance with the process of my earlier patent include the esters of phosphorous acid, including the alkyl, aryl, alk-aryl, and heterocyclic phosphites such as ethyl phosphite, propyl phosphite, butyl phosphite, amyl phosphite, cyclohexyl phosphite, phenyl phosphite, cresyl phosphite, xylenyl phosphite, naphthyl phosphite, ethyl phenyl phosphite, propyl phenyl phosphite, butyl phenyl phosphite, amyl phenyl phosphite, cresyl phenyl phosphite, naphthyl phenyl phosphite, ethylhexyl phosphite, furfuryl phosphite, pyridyl phosphite and the like. Esters other than the neutral or triesters may also be utilized, for example, mono- and di-esters such as mono-amyl dihydrogen phosphite, dicresyl hydrogen phosphite, mono-phenyl dihydrogen phosphite, dibutyl hydrogen phosphite and the like.

Other organic compounds of trivalent phosphorus which may be employed in the practice of the method of my earlier patent are the phosphines such as tributyl phosphine, triamyl phosphine, triphenyl phosphine, and the alk-aryl phosphines, i. e., butyl phenyl phosphine and the like. The amides of phosphorous acid may also be utilized, for example, mono- and dibutyl

phosphorous acid amide, mono- and diamyl phosphorous acid amide, the aryl amides such as phenyl phosphorous acid amide, toluyl phosphorous acid amide, and the like.

5 Any of the foregoing compounds may also be used in the practice of the method of my present invention, which likewise involves reacting a hydrocarbon lubricating oil with an organic compound of trivalent phosphorus, but I generally use an alk-aryl phosphite and most preferably, an alk-aryl phosphite of the formula,



15 in which R may be any aliphatic hydrocarbon group such as ethyl, propyl, butyl, amyl, hexyl, heptyl, octyl, etc., which may itself be further substituted. Exemplary of compounds in which 20 R is further substituted are the acyl dicresyl phosphites such as ethanoyl (acetyl) dicresyl phosphite, propanoyl (propionyl) dicresyl phosphite, and the mixed alk-aryl dicresyl phosphites as amyl propyl phenyl dicresyl phosphite, amyl heptyl phenyl dicresyl phosphite, propyl cresyl ethyl dicresyl phosphite, butyl phenoxy propyl dicresyl phosphite, octyl phenoxy ethyl dicresyl phosphite, etc. Compounds of the type 25 of the last two compounds mentioned, that is, mixed alk-aryl dicresyl phosphites in which the aryl group is oxy substituted, are particularly suited for use in the execution of the present invention.

According to my earlier process, the mixture 30 of hydrocarbon oil and organic compound of trivalent phosphorus are blown with air or other oxygen-containing gas throughout the course of the thermal treatment, which is continued until the formation of sludge occurs in the mixture. 35 I have now found that a lubricating oil of even more superior characteristics, particularly as regards oxidation stability and tendency toward sludge formation, is produced when the thermal treatment is conducted in the absence of air or other oxidizing gas artificially introduced, and if the treatment is not continued to the extent of causing the formation of a separable sludge. 40 As a result of such modified treatment, the soluble phosphorus-containing compounds formed in the oil are either of a nature dissimilar to the soluble phosphorus compounds formed in an oil treated by my other process or, if they are the same compounds, they are formed in 45 greatly increased and therefore more effective quantities.

In carrying out the method of the present invention, hydrocarbon lubricating oil is admixed with an organic compound of trivalent phosphorus, which is preferably an alk-aryl tricresyl phosphite, and most suitably an alk-ar oxy alkyl tricresyl phosphite, such as octyl phenoxy ethyl tricresyl phosphite, in an amount varying from 0.25% to 50% by volume. This mixture in the form of a substantially homogeneous solution is then subjected to heating to a temperature of from 300° F. to 500° F., and preferably from 325° F. to 425° F., for a period of time which may vary from 1 hour or less to 40 or 50 hours or more, depending, inter alia, upon the quantity of phosphorus compound which was mixed with the oil and the operating temperature. In general, the higher the percentage of phosphorus compound in the oil, the longer the treatment time necessary to produce an oil of the desired characteristics. For that reason I usually prefer to treat an oil containing not substantially more than 10% of the phosphorus compound in which event the treatment period usually does not exceed 20 hours. It is to be emphasized that by my new method, no haze or insoluble matter is allowed to form in the oil although it may become slightly darker in color. In order to insure that the treatment will not be extended to the point at which sludge formation occurs, a test sample may be first run and the point of sludge formation noted. I prefer to carry the treatment of the oil very close to the sludge formation point as indicated by the test sample.

The treated oil may be used for lubrication purposes per se, but is usually diluted with 10 to 20 parts of untreated oil prior to such use.

Hydrocarbon oils from various sources have been treated according to the method of the present invention, and all have been found amenable thereto, the degree of oxidation inhibition being practically the same in all cases. My process is particularly valuable as applied to the treatment of paraffin base oils or oils in which the number and amount of naphthenic components has been reduced as by solvent extraction. Such oils are particularly prone toward oxidation and the corrosion of bearing surfaces, especially in motors operated at speeds conducive to crank case temperatures of the order of 275° F. or higher.

The treatment according to the invention may be carried out in vessels of varying dimensions; however, with some oils, increasing the area of the oil exposed to the atmosphere, may slightly decrease the time of treatment necessary to produce a satisfactory product.

The phosphorus-containing compounds formed in the treated oil not only inhibit oxidation of the oil, but also increase the film-strength thereof and to a degree not exceeded by the phosphorus compounds formed by my other method.

Oil treated in accordance with the invention and containing substantial quantities of the oxidation, sludging or corrosion inhibitors or film-strengthening agents, as the case may be, produced by the treating reaction described, may be subjected to selective solvent extraction whereby these inhibitors or film-strengthening agents are concentrated in an oil fraction produced by the solvent extraction. In the extraction, solvents such as aliphatic alcohols, esters, ketones, phenols, furfural, nitrobenzene and chlorex may be used. Also, oils containing substantial quantities of the inhibitors or film-strengthening agents may be contacted with an adsorbent medium such as fuller's earth, activated clay, silica

gel, bauxite or the like, whereby the said inhibitors or agents are adsorbed from the oil and concentrated in the adsorbent. The inhibitors or agents may then be recovered, as concentrates, 5 by washing the adsorbent with a solvent for the inhibitors or agents.

My invention may be further illustrated by the following examples which are not to be construed as limiting the scope thereof:

- 10 (1) Hydrocarbon oil having a Saybolt Universal viscosity of 315 seconds at 100° F., an A. P. I. gravity of 29.0°, and an A. S. T. M. color of 3 was admixed with about 1.5% (by volume) of octyl phenoxy ethyl tricresyl phosphite, and heated at 340° F. for 16 hours without air blowing or other agitation. During the thermal treatment, the oil became slightly darker in color, but no haze or other insoluble material was formed. The treated oil was thereafter blended with 14 15 times its volume of untreated oil of the same characteristics as above, making a final concentration of the additive of 0.1%. A sample of the blended oil was subjected to an oxidation test comprising heating 100 cc. of the oil at 340° F. 20 for 96 hours, air being blown through the sample at a rate of 3 liters per hour. Despite the length of the test period, only 36 mg. of sludge formed in the oil for each 10 gm. of oil subjected to the test. When a sample of the untreated oil was 25 subjected to the same test, 240 mg. of sludge formed in the oil per each 10 gm. of the oil.
- (2) A hydrocarbon oil having a Saybolt Universal viscosity of 315 seconds at 100° F., an A. P. I. gravity of 29.5°, and an A. S. T. M. color 30 of 2½, the oil being from a different source than that used in Example 1, was treated in a like manner. A sample of a blend of the concentrate was untreated oil (same oil as used to prepare the concentrate), which blend contained the inhibitor in a concentration of 0.1%, was subjected to the 96-hour oxidation test together with a sample of the same oil containing no inhibitor. 48 mg. of sludge formed in the uninhibited oil per each 10 gm. of oil, while only 3 mg. formed 35 in the blend per each 10 gm. thereof.
- (3) Cadmium-silver test bearings, when immersed in the blended inhibitor-containing oils of Examples 1 and 2 for 44 hours at 340° F., air being blown through the oil at a rate of 3 liters per 100 cc. per hour, showed no loss in weight, whereas similar bearings, tested in the untreated oils, showed a corrosion loss of 60 mg. in weight.
- The organic compound of trivalent phosphorus employed as the inhibitor in the foregoing examples is a water-insoluble reaction product of tricresyl phosphite and octyl phenoxyethanol. It may be prepared by admixing tricresyl phosphite with octyl phenoxyethanol and thereafter bringing the mixture to a temperature sufficient to cause reaction of the ingredients, whereby there is introduced into the tricresyl phosphite at least one octyl phenoxyethanol group. The mol ratio of tricresyl phosphite to octyl phenoxyethanol employed may vary from 1:1 to 1:2.5, and is preferably of the order of 1:1.4. The reactants may be heated at atmospheric pressure under a reflux condenser to a temperature sufficient to effect reaction, for example, temperatures of the order of from 200° F. to 500° F., and the resulting oil-soluble water-insoluble reaction product may be separated from the by-products of the reaction by distillation under reduced pressure, or by recrystallization from a suitable solvent, or by washing with a solvent having selective solvent power for either the reaction product or the undesirable

by-products. Preferably, however, the reaction between the ingredients is carried on at elevated temperatures of the order of from 200° F. to 350° F. under reduced pressures of the order of 10 mm. or less. The reaction product produced may be regarded as a complex ester of phosphorous acid which may or may not contain unreacted octyl phenoxyethanol. Such reaction product has a wider range of utility and effectiveness as an inhibitor and the like than the simple ester, i. e., tricresyl phosphite from which it is prepared.

Although I have done most of my work using octyl phenoxy ethyl dicesyl phosphite as the oxidation inhibiting or film-strengthening agent, it is to be understood, as brought out in the forepart hereof, that other organic compounds of trivalent phosphorus may be employed, including the alkyl phosphites, alkyl-aryl phosphites, mixed alkyl-aryl phosphites, organic phosphines, phosphorous acid amides and the like.

It should also be stated that the treatment described hereinabove is adapted to viscous hydrocarbon oils, i. e., lubricating oils or lubricating oil stocks produced by distillation, acid treatment, clay treatment or solvent treatment, regardless of the source of the crude oils from which the lubricating oils or stocks may have been derived.

The improved oils, produced in accordance with the present invention, may be employed in the manufacture of thickened oils or greases or may be blended with fatty oils, synthetic esters, fatty acids, chlorinated or sulfurized compounds, alkali or heavy metal soaps or other agents utilized in the production of compounded lubricants.

I claim:

1. The method of producing an improved lubricating oil which comprises adding to a hydrocarbon oil, containing lubricating oil components, an organic compound of trivalent phosphorus, subjecting the resulting mixture, in the absence of an oxidizing agent introduced from an extraneous source, to a heat treatment at a temperature and for a period of time sufficient to cause the formation of soluble phosphorus-containing reaction products, said treatment being discontinued prior to the formation of an insoluble sludge.

2. The method of producing an improved lubricant which comprises forming a concentrate of an organic compound of trivalent phosphorus in a hydrocarbon oil containing lubricating oil components, heating the concentrate, in the absence of an oxidizing agent introduced from an extraneous source, at a temperature and for a period of time sufficient to cause the formation of soluble phosphorus-containing reaction products but insufficient to cause the appearance of insoluble sludge, and blending the thus treated concentrate with a major portion of hydrocarbon oil.

3. The method of producing an improved lubricating oil which comprises adding to a hydrocarbon oil, containing lubricating oil components, an organic compound of trivalent phosphorus, subjecting the resulting mixture, in the absence of an oxygen-containing gas introduced from an extraneous source, to a heat treatment at a temperature of from 300° F. to 500° F. for a period of time sufficient to cause the formation of soluble phosphorus-containing reaction products but insufficient to cause the appearance of insoluble sludge.

4. The method of producing an improved lu-

bricant which comprises forming a concentrate of an organic compound of trivalent phosphorus in a hydrocarbon oil containing lubricating oil components, heating the concentrate at a temperature between 300° and 500° F., in the absence of an oxygen-containing gas introduced from an extraneous source, for a period of time sufficient to cause the formation of soluble phosphorus-containing reaction products but insufficient to cause the appearance of insoluble sludge, and blending the thus treated concentrate with a major portion of hydrocarbon oil.

5. The method of producing an improved lubricating oil which comprises adding to a hydrocarbon oil, containing lubricating oil components, from 0.25% to 50% of an organic compound of trivalent phosphorus, subjecting the resulting mixture, in the absence of an oxygen-containing gas introduced from an extraneous source, to a heat treatment at a temperature of from 300° F. to 500° F. for a period of time sufficient to cause the formation of soluble phosphorus-containing reaction products but insufficient to cause the appearance of insoluble sludge.

6. The method of producing an improved lubricant which comprises forming a concentrate of an organic compound of trivalent phosphorus in a hydrocarbon oil including lubricating oil components, said concentrate containing from 0.25% to 50% of the said compound, heating the concentrate at a temperature between 300° F. and 500° F., in the absence of an oxygen-containing gas introduced from an extraneous source, for a period of time sufficient to cause the formation of soluble phosphorus-containing reaction products but insufficient to cause the appearance of insoluble sludge, and blending the thus treated concentrate with a major portion of hydrocarbon oil.

7. The method of producing an improved lubricating oil which comprises adding to a hydrocarbon oil, containing lubricating oil components, an ester of phosphorous acid, subjecting the resulting mixture, in the absence of an oxidizing agent introduced from an extraneous source, to a heat treatment at a temperature and for a period of time sufficient to cause the formation of soluble phosphorus-containing reaction products, said treatment being discontinued prior to the formation of an insoluble sludge.

8. The method of producing an improved lubricant which comprises forming a concentrate of an ester of phosphorous acid in a hydrocarbon oil containing lubricating oil components, heating the concentrate, in the absence of an oxidizing agent introduced from an extraneous source, at a temperature and for a period of time sufficient to cause the formation of soluble phosphorous-containing reaction products but insufficient to cause the appearance of insoluble sludge, and blending the thus treated concentrate with a major portion of hydrocarbon oil.

9. The method of producing an improved lubricating oil which comprises adding to a hydrocarbon oil, containing lubricating oil components, a mixed alkyl-aryl ester of phosphorous acid, subjecting the resulting mixture, in the absence of an oxidizing agent introduced from an extraneous source, to a heat treatment at a temperature and for a period of time sufficient to cause the formation of soluble phosphorus-containing reaction products, said treatment being discontinued prior to the formation of an insoluble sludge.

10. The method of producing an improved lu-

bricant which comprises forming a concentrate of a mixed alkyl-aryl ester of phosphorous acid in a hydrocarbon oil containing lubricating oil components, heating the concentrate, in the absence of an oxidizing agent introduced from an extraneous source, at a temperature and for a period of time sufficient to cause the formation of soluble phosphorous-containing reaction products but insufficient to cause the appearance of insoluble sludge, and blending the thus treated concentrate with a major portion of hydrocarbon oil.

11. The method of producing an improved lubricating oil which comprises adding to a hydrocarbon oil, containing lubricating oil components, an alk-aroxy alkyl dicesyl phosphite, subjecting the resulting mixture, in the absence of an oxidizing agent introduced from an extraneous source, to a heat treatment at a temperature and for a period of time sufficient to cause the formation of soluble phosphorus-containing reaction products, said treatment being discontinued prior to the formation of insoluble sludge.

12. The method of producing an improved lubricant which comprises forming a concentrate of an alk-aroxy alkyl dicesyl phosphite, in a hydrocarbon oil containing lubricating oil components, heating the concentrate, in the absence of an oxidizing agent introduced from an extraneous source, at a temperature and for a period of time sufficient to cause the formation of soluble phosphorus-containing reaction products but insufficient to cause the appearance of insoluble sludge, and blending the thus treated concentrate with a major portion of hydrocarbon oil.

13. The method of producing an improved lubricating oil which comprises adding to a hydrocarbon oil, containing lubricating oil components, octyl phenoxy ethyl dicesyl phosphite, subjecting the resulting mixture, in the absence of an oxygen-containing gas introduced from an extraneous source, to a heat treatment at a temperature of from 300° F. to 500° F. for a period of time sufficient to cause the formation of soluble phosphorus-containing reaction products but insufficient to cause the appearance of insoluble sludge.

14. The method of producing an improved lubricant which comprises forming a concentrate of octyl phenoxy ethyl dicesyl phosphite in a hydrocarbon oil containing lubricating oil components, heating the concentrate at a temperature between 300° F. and 500° F., in the absence of an oxygen-containing gas introduced from an extraneous source, for a period of time sufficient to cause the formation of soluble phosphorus-containing reaction products but insufficient to cause the appearance of insoluble sludge, and

blending the thus treated concentrate with a major portion of hydrocarbon oil.

15. The method of producing an improved lubricating oil which comprises adding to a hydrocarbon oil, containing lubricating oil components, from 0.25% to 50% of octyl phenoxy ethyl dicesyl phosphite, subjecting the resulting mixture, in the absence of an oxygen-containing gas introduced from an extraneous source, to a heat treatment at a temperature of from 300° F. to 500° F. for a period of time sufficient to cause the formation of soluble phosphorus-containing reaction products but insufficient to cause the appearance of insoluble sludge.

16. The method of producing an improved lubricant which comprises forming a concentrate of octyl phenoxy ethyl dicesyl phosphite in a hydrocarbon oil including lubricating oil components, said concentrate containing from 0.25% to 50% of the said phosphite, heating the concentrate at a temperature between 300° F. and 500° F., in the absence of an oxygen-containing gas introduced from an extraneous source, for a period of time sufficient to cause the formation of soluble phosphorus-containing reaction products but insufficient to cause the appearance of insoluble sludge, and blending the thus treated concentrate with a major portion of hydrocarbon oil.

17. The method of producing an improved lubricating oil which comprises adding to a hydrocarbon oil, containing lubricating oil components, from 0.25% to 10% of octyl phenoxy ethyl dicesyl phosphite, subjecting the resulting mixture, in the absence of an oxygen-containing gas introduced from an extraneous source, to a heat treatment at a temperature of from 325° F. to 425° F. for a period of time sufficient to cause the formation of soluble phosphorus-containing reaction products but insufficient to cause the appearance of insoluble sludge.

18. The method of producing an improved lubricant which comprises forming a concentrate of octyl phenoxy ethyl dicesyl phosphite in a hydrocarbon oil including lubricating oil components, said concentrate containing from 0.25% to 10% of the said octyl phenoxy ethyl dicesyl phosphite, heating the concentrate at a temperature between 325° F. and 425° F., in the absence of an oxygen-containing gas introduced from an extraneous source, for a period of time sufficient to cause the formation of soluble phosphorus-containing reaction products but insufficient to cause the appearance of insoluble sludge, and blending the thus treated concentrate with a major portion of hydrocarbon oil.

WILLIAM SCHREIBER.

## CERTIFICATE OF CORRECTION.

Patent No. 2,365,974.

December 26, 1944.

WILLIAM SCHREIBER.

It is hereby certified that error appears in the printed specification of the above numbered patent requiring correction as follows: Page 2, second column, line 38, for "was untreated" read --with untreated--; and that the said Letters Patent should be read with this correction therein that the same may conform to the record of the case in the Patent Office.

Signed and sealed this 20th day of March, A. D. 1945.

Leslie Frazer

(Seal)

Acting Commissioner of Patents.